

Aug. 24, 1948.

F. E. WILLIAMS

2,447,927

LUMINESCENT ZINC FLUORIDE

Filed Oct. 17, 1945



INVENTOR.  
*Ferd E. Williams*

BY

*Charles McClain*  
ATTORNEY

## UNITED STATES PATENT OFFICE

2,447,927

## LUMINESCENT ZINC FLUORIDE

Ferd E. Williams, Princeton, N. J., assignor to  
 Radio Corporation of America, a corporation of  
 Delaware

Application October 17, 1945, Serial No. 622,823

2 Claims. (Cl. 252—301.6)

**1**

This invention relates to materials capable of fluorescing under excitation of agents, such as cathode rays, with a relatively long decay rate in luminescence when the excitation is removed.

In phosphors of the type disclosed, the intensity of luminescence is given by the equation  $I=At^{-n}$ , where  $A$  is a constant depending upon the particular ingredients and excitation intensity,  $t$  is time and  $n$  is a variable also dependent upon the ingredients of the mixture, particularly the activator used.

It is an object of this invention to provide a phosphor of good efficiency and a relatively slow decay rate.

Another object is to provide a phosphor of zinc fluoride with an activator capable of varying the decay rate.

Other objects of the invention will appear in the following specification, reference being had to the drawing, in which the single figure of the drawing contains graphs illustrating the performance of the improvement, the abscissas representing time in seconds in linear scale and the ordinates representing intensity of luminescence in logarithmic scale.

Zinc fluoride with manganese activator has been found to be particularly efficient in radar and similar uses because of its characteristic decay rate. The luminescence continues for a sufficient time to satisfactorily show the trace of moving objects and then blanks out suddenly. Such a phosphor is disclosed in the application of Maggio Banca, filed April 19, 1945, Serial No. 589,269.

I have found that zinc fluoride, when activated by columbium (also known as niobium), has a quite broad spectrum with a peak at 4700 Å. and that  $n$  in the equation  $I=At^{-n}$  can be varied from 0.8 to 1.2 by increasing the columbium gram mole content from  $ZnF_2:0.0008$  Cb to  $ZnF_2:0.03$  Cb. This control of the decay is an important advantage.

In the drawing, curve 1 shows the decay characteristic of the zinc fluoride phosphor when 0.0008 gram mole of columbium activator is used

**2**

to each gram mole of zinc fluoride. Curve 2 shows the characteristic with 0.03 gram mole of columbium per gram mole of zinc fluoride. It will be apparent that wide control of the decay rate can be obtained by varying the columbium content.

The phosphor may be prepared by adding C. P. concentrated hydrofluoric acid to zinc oxide and columbium of the desired content, either as a salt such as  $CbSO_4x(OH)y$ , or as a metal. However, the use of metallic columbium, preferably in powder form, is preferred, as the sulphate or other anion decreases the efficiency of the phosphor. The materials, after thorough mixing, are evaporated to dryness by heating for about one-half hour at from 500° C. to 900° C. in a relatively neutral atmosphere.

The columbium activator is thought to exist in the fluoride crystal lattice as the oxide and not as the fluoride, since the latter boils at 229° C.

Having described my invention, what I claim is:

1. A phosphor consisting of zinc fluoride and an activator of columbium having a gram mole ratio to the zinc fluoride of substantially 0.0008 to 1.
2. A phosphor consisting of zinc fluoride and columbium activator in the ratio of 0.0008 to 0.03 gram mole of columbium to one gram mole of zinc fluoride.

FERD E. WILLIAMS.

## REFERENCES CITED

- 35 The following references are of record in the file of this patent:

## UNITED STATES PATENTS

- |           |         |               |
|-----------|---------|---------------|
| 40 Number | Name    | Date          |
| 2,049,765 | Fischer | Aug. 4, 1936  |
| 2,226,407 | McKeag  | Dec. 24, 1940 |

## OTHER REFERENCES

- 45 Chem. Abstracts, vol. 18, page 2287.